

## UNITED STATES PATENT OFFICE

1,956,025

## PROCESS FOR REVIVIFYING FILTERING MATERIALS

John D. Haseman, Linton, Ind.

No Drawing. Application October 15, 1930,  
Serial No. 489,008

2 Claims. (Cl. 252—2)

The invention relates to a method of revivifying bleaching materials, and it has for its object to provide a novel method whereby spent fine fuller's earth, processed bentonite and the like 5 may be revivified to yield a more efficient decolorizer with little or no loss of the fine particles and with a minimum expenditure of energy.

The contact method of decolorizing heavy acid stocks as now practiced leaves a gasoline-steam 10 washed fine loose 200 mesh spent material which on being heated to burn out the injurious products blow away by the rapid evaporation of the adsorbed gasoline and consequent tumbling about of the material in burning out the carbon evolved 15 from the lubricating oil and the adsorbed color compounds. The loss is so great that dust collectors are required to catch the particles carried away before they have been properly revivified. Hence with present practices it is impossible to 20 burn out fine spent bleaching materials at a uniform and efficient temperature.

I have discovered that when 25 to 50% by weight of water is mixed with the fine spent bleaching material that it sticks together so that 25 the rapid evaporation of gasoline or burning out of the lubricating oil will not carry away any of the fine bleaching material, and that the adhered particles can all be burned out at the same temperatures.

30 My preference in practice is to mix the dry fine loose bleaching material with fifty percent of water and spread it uniformly on a metal conveyor running through a hooded lead heated furnace which has increasing temperatures. The

hottest end of the furnace should be around 900 degrees Fahr. and has provisions for admitting steam as well as the escape of the final carbonizing products. This low temperature carbonizing furnace should preferably be closed and in at least 30 three sections having escape openings or hoods.

This preference in practice will not only prevent loss of fine particles and destroy the injurious catalyzed products of the spent clay but will 65 also activate much of the carbonized material and thereby yield a more efficient revivified material.

The above description is not to be taken as limiting my invention, but is merely illustrative of 70 the best method of carrying it out. As will be understood by those skilled in the art, many modifications can be made within the spirit of my invention which I claim to be.

I claim:

1. Process which consists in mixing spent 75 bleaching material with water to make it slightly plastic, driving off the more volatile materials with low temperatures and driving off the injurious catalyzed products at a dull red heat in the absence of air.

2. Process which consists in mixing spent 80 bleaching material with water to make it slightly plastic, driving off the more volatile material with low temperatures, driving off the injurious catalyzed products at a temperature of dull red heat, 85 and activating the retained carbon in absence of air and the presence of steam.

JOHN D. HASEMAN.

35

95

40

100

45

105

50

110

55